

2,812,858

## PROCESS FOR RECOVERY OF PHOSPHATE MINERALS

Homer E. Uhland, Lakeland, Fla., assignor to International Minerals & Chemical Corporation, a corporation of New York

No Drawing. Application November 29, 1954,  
Serial No. 471,890

11 Claims. (Cl. 209—166)

This invention relates to a process for beneficiation of ores. More particularly it relates to a process for separating phosphate material from gangue constituents of phosphate ore such as Florida pebble phosphate ore bodies. Still more particularly it relates to a process for the recovery of phosphate values normally lost in the tailings from the amine flotation stage of the flotation process.

In the processing of minerals such as pebble phosphate ore bodies, generally speaking, the material is mined from the natural deposit and transferred to washers and then to flotation plants in which latter stages the material is treated in aqueous slurry form. This slurry contains sizeable amounts of silica, so-called colloidal phosphates, and clays normally delineated as slimes, as well as other gangue materials. In the flotation operation the phosphate is recovered in as pure a form as possible and is substantially free of slimes. In a flotation process the phosphate particles must be of such a size that they may be economically treated.

As an initial step in obtaining a flotation slurry, the ore material is subjected to a preliminary washing operation wherein a sizable quantity of the coarse phosphatic values are removed by a screen operation which produces a pebble product containing all of the +1 mm. values. The —1 mm. values containing the phosphatic particles, silica particles, and the slimes as a slurry must be further processed to give maximum recovery of the granular material and substantially complete removal of the slime material which if allowed to remain would adversely affect the subsequent concentration process, i. e., silica removal.

A rough separation of the slime material may be accomplished in a number of ways. As practiced commercially in the phosphate fields of Florida, recourse is taken to a hydro-separation or hydrocyclone process. The overflow from this hydroseparator or classification system is withdrawn and sent to a settling or slime pond. This overflow is made up chiefly of suspended clay and extremely fine particles of phosphate, i. e., particles of a sufficient degree of fineness that they could not be economically recovered at any subsequent step of the process. This separation is commonly made, in the phosphate field, at approximately 150 or 200 mesh. The coarser fraction, essentially —1 mm. and +150 mesh, is separately withdrawn. Following removal of this fraction, it is sized further; usually by hydraulic classification or screening at about 35 mesh to about 48 mesh. The coarser fraction (i. e. —1 mm. +35 mesh) is then treated for removal of the phosphate values on agglomerate tables, spirals, belts, underwater screens or by froth flotation. The finer fraction (i. e. —35+150 mesh) is then subjected to froth flotation operations.

In the froth flotation operation reagents are employed to float selectively a desired constituent of the ore. If the desired constituent is phosphate, then such reagents as fuel oil, kerosene along with long chain fatty acids and caustic soda, fatty acid soaps and the like are used.

In general, the concentrates from rougher flotation steps are subjected to scrubbing with chemical agents to remove flotation reagents and then to secondary flotation operations which float the minor constituents of the concentrates. In the case of phosphate flotation, the reagents utilized in the secondary flotation are amines derived from long chain fatty acids or salts thereof such as the acetate salt. This secondary flotation operation floats the minor constituent of the concentrate, which at this stage of phosphate flotation procedure is silica. Amines and their salts, while effective as flotation reagents for silica, are nevertheless not highly selective, i. e., are not effective depressants for phosphates. As a consequence, considerable quantities of phosphate material are floated together with the silica, and this phosphate material is lost in the silica tail which is sent to waste.

Presence of the amine reagent has proven an effective barrier to re-reagentizing the silica tail with agents which would be selective for phosphate flotation. Further, the removal of the amine reagents by chemical means has proven expensive and entirely unsatisfactory.

It is a primary object of this invention, therefore, to overcome the shortcomings and disadvantages of the process heretofore in use.

It is a further object of this invention to teach a process wherein the secondary reagents are removed so that the tail fractions may be resubjected to flotation with reagents selective to the desired constituents of the concentrate.

It is still another object of this invention to provide a process wherein amine reagents used in the secondary flotation operations for phosphate are effectively removed from the tail fraction.

It is still another object of this invention to provide a process wherein higher recovery of phosphate is attained due to the removal of amine reagents, which then permits the reworking of the tail to recover phosphate constituents heretofore lost to waste.

These and other objects of the invention will be obvious to those skilled in the art from a study of the process hereinafter outlined in detail.

Now it has been discovered that the amine reagents present on products recovered in amine flotation operations, which amines heretofore have not been susceptible of economic removal and which interfere with subsequent conditioning of products with anionic reagents and with subsequent attempts at flotation for improvement of the recovery of a desired component, can be cheaply and effectively removed by mixing the amine flotation product in slurry form with so-called slime materials and agitating the mixture. During agitation the amine reagents are transferred to the slime particles. The mixture is next subjected to wet classification separations to remove the slime material from the flotation product solids. The deslimed solids may then be conditioned with anionic reagents for flotation, and the desired components which would be lost as a result of discarding the amine flotation product may be recovered by flotation in a concentrated form.

More in detail, the method as applied to the processing of Florida pebble phosphate ore comprises, generally speaking, transfer of the matrix as mined from the natural deposit in slurry form. This slurry contains sizeable amounts of silica clay and miscellaneous gangue material, as well as phosphate particles in various forms and particle size. Phosphate particles having a diameter of approximately +1 mm. are removed from the slurry by a washing and screening operation and marketed as pebble. The —1 mm. material is subjected to hydroseparation or other wet classification operation. The overflow product from the hydroseparator constitutes the so-called slimes of the system and is made up chiefly of dissolved and suspended clay and so-called colloidal phosphate, i. e., phos-

phate of a particle size of the same order of magnitude as the suspended clays.

Underflow solids from the hydroseparation step are subjected to beneficiation processes such as froth flotation to free the phosphate of silica and minor amounts of gangue material in order to produce a phosphate concentrate, preferably of about 74% to about 78% bone phosphate of lime content if the character of the rock is such as to permit production of such a grade.

In the froth flotation operation reagents are employed depending upon the constituent which is to be floated. In a typical phosphate operation the first stage flotation utilizes carboxyl-containing negative ion agents such as are found in the mixture of fuel oil, kerosene, and long chain fatty acids as well as caustic soda. This mixture characterized by the fatty acids generally denominated anionic agent flotation froths up and floats away a predominantly phosphate material as concentrate.

An effective way to upgrade the phosphate concentrate further is to subject it to a cationic or positive ion agent flotation, which process floats the silica and leaves a phosphate concentrate as the underflow product. Before conditioning the phosphate concentrate with cationic agents, the anionic agent or agents are removed from the first concentrate by scrubbing it with about a 20% sulfuric acid solution. The language "scrubbing" as used in wet mineral processing means agitating the solids in slurry form generally in a solids content of about 45% to about 75% solids. After scrubbing the phosphate concentrate, the acid solution is removed in dewatering and washing steps. Concentrate solids are then slurried in water and conditioned with amines or salts of amines derived from long chain fatty acids such as primary monoamines derived from hydrogenated tallow, fatty acids or from soya fatty acids, N-dodecylamine, N-hexadecylamine, etc.; diamines or salts of diamines such as lauryl fatty diamine or soya fatty diamine acetate.

Under current operating procedures, the amine tail product is sent to waste with from about 10% to about 45% bone phosphate of lime content. In a plant processing 500 tons per hour of underflow solids from the hydroseparator this percentage of B. P. L. material constitutes an appreciable loss. In the new process as applied to phosphate ore processing, this amine tail product generally in slurry form is mixed with the overflow slimes from the above described hydroseparation operation. The invention at this stage will immediately suggest two modes of operation. In the first modification this amine tail product is delivered to the above described hydroseparation operation wherein slimes are removed on a continuous recycle basis. In the second and preferred mode of operation, the amine tail product is mixed with overflow slimes in proportions giving a resultant slurry having about 1/2% to about 5% by weight of slime solids. Slimes are generally incorporated into the amine tails product by adding between about 10 and about 100 gallons per minute of slime slurry which corresponds to the addition of approximately 2 pounds to approximately 20 pounds of slime solids per ton of amine tail solids. The resultant slurry is agitated at about 50% to about 70% solids content for between about 30 seconds and about 180 seconds, with an optimum period of about 90 seconds to about 130 seconds preferred. Slimes which preferentially take up or adsorb the amine reagent are removed from contact with the tail solids by classification or hydroseparation or hydrocyclone operations.

Deslimed silica tail material is next conditioned with anionic reagents, for example, the tall oil kerosene mixture used for the flotation of the original phosphate concentrate together with fuel oil and caustic soda. Flotation of the conditioned tail product gives a recovery of about 90% to about 98% of the phosphate in the tail. This secondary concentrate can be refloated to produce a product of between about 2% to about 8% acid insoluble

material combinable with the initial phosphate concentrate.

The amount of negative and positive ion agents which are employed in the flotation steps which are an integrated part of the instant novel process may vary according to the phosphatic or silicious content of the ore. The amount of negative ion agent which is employed to produce a flotation concentrate may vary over a fairly wide range, but between about 0.4 pound and about 2 pounds of negative ion agent per ton of solids in the flotation pulp has been found to be particularly advantageous. When conducting a flotation operation in the presence of positive ion agent, for example, long chain aliphatic amines or their water soluble acid addition salts, the amount of such reagent may vary over fairly wide limits but between about 0.2 pound and about 1 pound of such reagent per ton of ore based upon the solids content of the reagentized pulp is conveniently employed. The amount of frothing and other agents, such as pine oil, kerosene, fuel oil, etc., which is optionally but generally present during flotation may also vary over fairly wide limits, between about 0.1 pound and about 1 pound per ton of solids in a flotation pulp. The type of reagent employed will be particularly effective within certain pH ranges, for example, the negative ion agents are generally effective in the alkaline pH range. Negative ion reagents selected from the group comprising fatty acids, resin acids, tail oil, naphthalene acids, soaps of these reagents, etc. are particularly effective when conducting a flotation operation at a pH in the range between about 7 and about 9. The invention is not limited to such reagents, but any reagent which has an affinity for phosphate values may be employed similarly. Reagents other than long chain aliphatic amines or their water soluble acid addition salts are effective at pH's in the range between about 3 and about 6. It will be obvious to those skilled in the art of flotation that the selectivity of any particular reagent or mixtures of several reagents is not usually sufficient to achieve a complete recovery of the desired component in any one flotation operation. It is, therefore, within the scope of the invention to recycle various pulp streams from any particular flotation operation whether this will be a rougher or a cleaner flotation.

The invention will be better understood from the following description and examples.

#### EXAMPLE I

A phosphate rock such as the type found in the phosphate pebble fields of central Florida is subjected to a washing operation in order to remove slimes and organic matter. The washed rock in an aqueous pulp is subjected to screening or hydraulic sizing operation whereby the larger particles of rock are segregated from material which is -35 mesh particle size. The material remaining after 50 the pebble has been removed, which consists of phosphate, clay, silica and the like, is further treated by hydroseparation to overflow the fine particles normally discarded from the system as slimes and to recover underflow particles which are then conditioned in an aqueous pulp containing about 60% solids with about one pound per ton of ore solids, the reagent comprising about 75% tall oil and about 25% kerosene. About 3 pounds of fuel oil is added to the mixture and sufficient caustic soda is added to give the mixture a pH in the range of between about 8.5 to 60 about 9.0. The resultant pulp is then subjected to a flotation operation at a solids content of about 30% by weight in a Denver laboratory machine and a float recovered containing approximately 60% tricalcium phosphate, the balance being silica and silicious gangue. This 65 phosphatic concentrate is scrubbed with about 2 pounds of sulfuric acid (60° Bé.) per ton of solids in order to remove the reagents therefrom. The acid-treated product is washed until it is substantially neutral and is then conditioned in an aqueous pulp with a mixture of long chain 70 aliphatic amines, the latter comprising a mixture of about 75

73% mono-octadecylamine and about 24% mono-hexadecylamine, together with small quantities of secondary and tertiary amines whose aliphatic groups contain between about 12 and about 18 carbon atoms. This reagent can be added in the form of an acid addition salt. The conditioned concentrate is then subjected to a flotation operation at a solids content of about 30% in a Denver laboratory flotation machine. The float product from this operation is a predominantly silica material, i. e., the product contains approximately 85% of the silica originally in the concentrate and has an approximately 15% bone phosphate of lime content.

#### EXAMPLE II

Amine reagent flotation tail (silica float product from Example I) was washed and watered. Equal portions of this washed product were conditioned in an aqueous pulp of approximately 60% solids with about 0.5 pounds of reagent per ton of silica product treated; the reagent comprising approximately 75% tall oil and 25% kerosene by weight. About 3 pounds of fuel oil and sufficient caustic soda was added to give the conditioned pulp a pH of between 8.5 to 9.0 in each instance. Each conditioned pulp was then subjected to flotation at a solids content of approximately 30% by weight in a Denver laboratory flotation machine to produce a flotation product and a phosphate concentrate product. The phosphate concentrate products produced were attrition scrubbed with about 2 pounds of sulfuric acid (60° Bé.) per ton of solids. This acid treated product was washed until it was substantially neutral and then conditioned in an aqueous pulp with a long chain aliphatic amine. The results obtained at two different amine concentrations are shown in the following table:

Table 1

| Product                    | Lbs. of Amine/Ton Treated | Percent B. P. L. | Percent Insol. |
|----------------------------|---------------------------|------------------|----------------|
| Phosphate Concentrate..... | 0.1                       | 32.66            | 58.20          |
| Tails.....                 |                           | 18.09            |                |
| Phosphate Concentrate..... | 0.2                       | 56.78            | 29.60          |
| Tails.....                 |                           | 19.70            |                |

From Table 1 it is clear that the amine tail phosphate concentrate is not susceptible to beneficiation to an economic product of industry.

#### EXAMPLE III

A portion of the amine flotation tail produced from Example I was mixed with slime material in proportions of 20 gallons of the hydroseparator overflow slurry to one ton of amine tail product. This corresponds to adding approximately 5 pounds of slime solids per ton of amine tail product. The solids mixture was agitated in an upright centrifugal mixer for two minutes and then deslimed by decantation. The dewatered solids were pulped with water and the aqueous pulp containing about 60% solids conditioned with about 0.5 pound of reagent per ton of solids the same as in Example II. The other accessory reagents and the subsequent flotation also were identical to that given the sample in Example II. The flotation product in this test was then given an amine flotation again identical to Example II. The results obtained on this test are shown in Table 2.

Table 2

| Product                    | Lbs. of Amine/Ton Treated | Percent B. P. L. | Percent Insol. |
|----------------------------|---------------------------|------------------|----------------|
| Phosphate Concentrate..... | 0.1                       | 75.17            | 8.00           |
| Tails.....                 |                           | 11.86            |                |
| Phosphate Concentrate..... | 0.2                       | 77.38            | 5.61           |
| Tails.....                 |                           | 13.87            |                |

The underflow product (phosphate concentrate) produced on these tests is acceptable to industry as an economic product.

Having thus fully described and illustrated the character of the invention, what is desired to be secured and claimed by Letters Patent is:

1. The method of removing cationic amine reagents from flotation separation products which were concentrated with the aid of said amine reagents which comprises mixing in slurry form the flotation product containing amine reagent and a slime material, agitating the mixture and subjecting the mixture to a wet classification operation to separate the slime material containing adsorbed amine reagents from the flotation products.
2. The method of removing cationic amine reagents from phosphate flotation products which were concentrated with the aid of amine reagents which comprises mixing the tail product containing amine reagent with slime material originally present in the ore, agitating the mixture and subjecting the mixture to a wet classification operation to separate the slime material containing adsorbed amine reagents from the tail product.
3. The method of improving the recovery of desired components of ores which are concentrated with the aid of cationic amine reagents comprising mixing in slurry form flotation operation products containing amine reagent with slime material, subjecting the slurry mixture to agitation and wet classification to separate slime material containing adsorbed amine reagent, subjecting the deslimed flotation product to a further flotation operation with anionic reagents and then subjecting the anionic reagent concentrate to flotation with cationic reagents to recover a concentrate of the desired component.
4. The method of improving the recovery of phosphate from Florida pebble phosphate ore which comprises mixing in slurry form the silica tail product obtained by means of amine reagent flotation with slime material originally present in the phosphate ore, subjecting the slurry mixture to agitation and wet classification to separate the slime material containing adsorbed amine reagent, subjecting the dewatered silica tail product to flotation with anionic reagents and then subjecting the anionic reagent concentrate to flotation with amine reagent to recover a phosphate concentrate.
5. In a process of concentrating minerals wherein an ore in a liberated state is first subjected to a flotation operation employing carboxyl-containing negative ion flotation agent and the flotation product is subjected to a second flotation operation employing nitrogenous positive ion flotation agent, the improvement comprising slurring a product from the nitrogenous positive ion flotation operation with slime material originally present in the ore, agitating the slurry mixture, removing the slime material from the flotation product by separative treatment, conditioning the deslimed product with carboxyl-containing negative ion reagent, subjecting the conditioned material to a froth flotation operation to recover a beneficiated fraction of the ore, and subjecting the beneficiated fraction to a final froth flotation operation.
6. The method of improving the recovery of desired components of ores which are concentrated with the aid of cationic amine reagents comprising mixing in slurry form flotation operation products containing amine reagent with slime material having a particle size of less than about 150 mesh to about 200 mesh standard screen size, subjecting the slurry mixture to agitation and wet classification to separate slime material containing adsorbed amine reagent, subjecting the deslimed flotation product to a further flotation operation with anionic reagents and then subjecting the anionic reagent concentrate to flotation with cationic reagents to recover a concentrate of the desired component.
7. The method of improving the recovery of desired components of ores which are concentrated with the aid

of cationic amine reagents comprising mixing in slurry form flotation operation products containing amine reagent with slime material having a particle size of less than about 150 mesh to about 200 mesh standard screen size, said slime material being added in quantities in the range between about 2 pounds and about 20 pounds of slime solids per ton of amine float product, agitating the slurry mixture for a period of about 90 seconds to about 130 seconds, subjecting the slurry mixture to wet classification to separate slime material containing adsorbed amine reagent, subjecting the deslimed flotation product to a further flotation operation with anionic reagents and then subjecting the anionic reagent concentrate to flotation with cationic reagents to recover a concentrate of the desired component.

8. The method of improving the recovery of phosphate from Florida pebble phosphate ore which comprises mixing in slurry form the silica tail product obtained by means of an amine reagent flotation with slimes removed from the ore prior to flotation, removing the slimes and conditioning the product with carboxyl-containing negative ion reagent, subjecting the conditioned material to a froth flotation operation to recover a phosphate fraction and subjecting the phosphate fraction to a final flotation operation with a long chain aliphatic amine-acid addition salt.

9. The method of improving the recovery of phosphate from Florida pebble phosphate ore which comprises wet classifying the ore to remove the low density fraction slimes therefrom, subjecting the slime free ore to a flotation operation at a pH in the range between about 7 and about 9 for the concentration of phosphate values with carboxyl-containing negative ion agent, subjecting the phosphatic concentrate to a silica flotation operation with a long chain aliphatic amine-acid addition salt, recirculating the amine flotation tail to the wet classification operation where the amine reagent is adsorbed by the slimes and floated away from the ore solids.

10. The process of recovering phosphate from Florida

pebble phosphate ore containing slime material wherein said ore is pulped with water and concentrates recovered by flotation, the steps comprising washing and sizing the ore to remove the +1 mm. size phosphate pebble, wet classifying the -1 mm. material to remove the -200 mesh standard screen size so-called slime material, subjecting the +200 mesh standard screen size fraction from said classification in a finely divided state to a flotation operation at a pH of between about 7 and about 9 for the concentration of phosphate values with carboxyl-containing negative ion agent, subjecting the phosphatic float to a silica flotation operation with a long chain aliphatic amine-acid addition salt, adding to the silica float a portion of the -200 mesh slime material, classifying the slurry mixture to remove the slime material containing adsorbed amine reagent from the amine tail solids, subjecting the amine tail solid to a flotation operation at a pH between about 7 and about 9 for the concentration of phosphate values with carboxyl-containing negative ion agent, and subjecting this fraction to a silica flotation operation with a long chain aliphatic amine-acid addition salt to recover a concentrate rich in phosphate material.

11. The method of improving the recovery of desired components of ores which are concentrated with the aid of cationic amine reagents comprising mixing in slurry form flotation separation products containing amine reagent with slime material, subjecting the slurry mixture to agitation and wet classification to separate slime material containing adsorbed amine reagent, and subjecting the deslimed flotation product to a further flotation operation with anionic reagents to recover a concentrate of the desired component.

35

References Cited in the file of this patent

UNITED STATES PATENTS

2,614,692 Lawyer \_\_\_\_\_ Oct. 21, 1952  
2,753,997 Duke et al. \_\_\_\_\_ July 10, 1956